# EUROPEAN PATENT SPECIFICATION

(11) **EP 1 812 187 B1**
(45) Date of publication and mention of the grant of the patent: **10.11.2010**
(21) Application number: 05783351.9
(22) Date of filing: 16.09.2005
(51) Int. Cl.: B22F 1/00, C22C 33/02

(54) **POWDER METAL COMPOSITION COMPRISING SECONDARY AMIDES AS LUBRICANT AND/OR BINDER**
SEKUNDÄRE AMIDE ALS SCHMIERMITTEL UND/ODER BINDEMITTEL UMFASSENDE PULVERMETALLZUSAMMENSETZUNG
COMPOSITION DE POUDRE METALLIQUE COMPRENANT DES AMIDES SECONDAIRES EN TANT QUE LUBRIFIANT ET/OU LIANT

(30) Priority: 17.09.2004 SE 0402239; 12.01.2005 SE 0500072
(43) Date of publication of application: 01.08.2007
(73) Proprietor: HÖGANÄS AB, 263 83 Höganäs (SE)
(72) Inventor: AHLIN, Åsa, S-263 37 Höganäs (SE); RAMSTEDT, Maria, S-252 52 Helsingborg (SE)
(74) Representative: Andersson, Mikael Per Robert
(86) International application number: PCT/SE2005/001343
(87) International publication number: WO 2006/031193

(56) References cited:
- EP-A- 1 197 975
- EP-A- 1 276 119
- EP-A1- 0 589 088
- WO-A1-92/18275
- WO-A1-96/25261
- WO-A1-97/43066
- US-A- 5 627 258
- DOROFEEV B. YU. ET AL.: "Formation of properties and interparticular concrescence of hotformed powder materials" , 1991, pages 789-794,

## Description

### Field of the invention

The present invention concerns a powder metal composition. Specifically the invention concerns a powder metal composition including a lubricant and/or binder comprising at least one secondary amide. The invention further concerns a method of producing a green body, a method of producing a bonded iron-based powder composition and use of the lubricant and/or binder.

### Background of the invention

Metal powders are used in industry for the manufacture of metal products by compacting the metal powder in a die under high pressures, ejecting the compact from the die and optionally sintering the product. In the majority of powder metallurgical (PM) applications a lubricant is comprised in the powder in order to provide the necessary lubrication action between powder particles during compaction and between the die and the compact during ejection from the die. Lubrication achieved by a lubricant included in the metal powder is referred to as internal lubrication in contrast to external lubrication, which is achieved by applying a lubricant to the walls of the die, wherein the powder is compacted. Insufficient lubrication during ejection results in excessive friction between the compact and the die resulting in high ejection energies and damage of die surfaces and product surfaces.

Internal lubrication is achieved by using special lubricants. Normally these lubricants are admixed with the iron or iron-based powder in the form of a powder. Some lubricants may also be used for binding additives, such as e.g. alloying elements, to the iron or iron-based particles. In these cases the lubricants thus work as binding agents and reduce or eliminate segregation of the additives during shipping and handling.

Commonly used lubricants for PM applications are metal soaps, such as lithium and zinc stearate. A disadvantage with this type of lubricant is that oxides of the metals in the lubricant contaminate the inside of the sintering furnace as a result of release of metals from the lubricant during sintering, another problem is that stains may be formed on the component after sintering. Another commonly used lubricant is ethylene bis stearamide (EBS). Stains may also be formed on the component after sintering when using this lubricant, but to a lesser extent compared with using e.g. zinc stearate. As lubricants strongly affect compacting and sintering properties of metal powders optimization of amount, composition and structure of the used lubricant is of vital importance to obtain high and consistent densities and good surface finishes of the produced parts.

### Objects of the invention

An object of the present invention is to provide a new powder metal composition comprising a lubricant and/or binder that reduces or eliminates the problems with high ejection forces and stained surfaces of the sintered parts.

Further objects of the invention are to provide a method of producing compacted products and sintered or heat treated parts, a method of producing a bonded powder metal composition and use of the lubricant and/or binder.

### Summary of the invention

These objects are accomplished by the powder metal composition defined in claim 1 comprising an iron based powder and a lubricant and/or binder comprising at least one secondary amide. The invention further concerns a method of producing a green body by subjecting the above mentioned composition to compaction.

The method of producing a bonded powder metal composition comprises: mixing an iron-based powder with at least one secondary amide and heating the mixture to a temperature above the melting point of the at least one secondary amide.

Additionally, the invention concerns the use of the at least one secondary amide as a lubricating and/or binding agent for iron-based powders, and its use for die wall lubrication.

### Detailed description of the invention

The lubricant and/or binder in the powder metal composition according to the invention is at least one secondary amide that may be defined by the general formula:

R₁-NH-CO-R₂,

wherein the R₁- and R₂-groups, which may be the same or different, are straight or branched, saturated or unsaturated aliphatic hydrocarbon groups.

Preferably, R₁ and R₂ independently include 10 to 24 carbon atoms.

Preferably R₁ and R₂ are selected from the group consisting of alkyl and alkenyl.

The alkyl groups may be chosen from decyl, undecyl, dodecyl, tridecyl, tetradecyl, pentadecyl, hexadecyl, heptadecyl, octadecyl, nonadecyl, eicosyl, heneicosyl, docosyl, tricosyl, tetracosyl.

The alkenyl groups may be chosen from decenyl, undecenyl, dodecenyl, tridecenyl, tetradecenyl, pentadecenyl, hexadecenyl, heptadecenyl, octadecenyl, nonadecenyl, eicosenyl, heneicosenyl, docosenyl, tricosenyl, tetracosenyl.

Examples of preferred secondary amides are shown in Table 1.

**Table 1**

| | | | | | General formula: R₁-NH-CO-R₂ | |
|---|---|---|---|---|---|---|
| R₁ no of C-atoms | R₂ no of C-atoms | R₁ | R₂ | Chemical name | Chemical structure | Common name |
| 18 | 15 | Octadecenyl | Pentadecyl | Octadecenylhexadecaneamide | CH₃(CH₂)₇HC=CH(CH₂)₈NHCO(CH₂)₁₄CH₄ | Oleyl palmitamide |
| 18 | 17 | Octadecyl | Heptadecyl | Octadecyloctadecaneamide | CH₃(CH₂)₁₇NHCO(CH₂)₁₆CH₃ | Stearyl stearamide |
| 18 | 17 | Octadecenyl | Heptadecyl | Octadecenyloctadecaneamide | CH₃(CH₂)₇HC=CH(CH₂)₈NHCO(CH₂)₁₆CH₃ | Oleyl stearamide |
| 18 | 17 | Octadecyl | Heptadecenyl | Octadecyloctadeceneneamide | CH₃(CH₂)₁₇NHCO(CH₂)₇HC=CH(CH₂)₇CH₃ | Stearyl oleamide |
| 18 | 17 | Octadecenyl | Heptadecenyl | Octadecenyloctadeceneneamide | CH₃(CH₂)₇HC=CH(CH₂)₈NHCO(CH₂)₇HC=CH(CH₂)₇CH₃ | Oleyl oleamide |
| 18 | 21 | Octadecyl | Heneicocenyl | Octadecyldococeneneamide | CH₃(CH₂)₁₇NHCO(CH₂)₁₁HC=CH(CH₂)₇CH₃ | Stearyl erucamide |
| 18 | 21 | Octadecenyl | Heneicocenyl | Octadecenyloctadeceneneamide | CH₃(CH₂)₇HC=CH(CH₂)₁₁NHCO(CH₂)₁₁HC=CH(CH₂)₇CH₃ | Oleyl erucamide |
| 22 | 17 | Dococenyl | Heptadecyl | Dococenyloctadecaneamide | CH₃(CH₂)₇HC=CH(CH₂)₁₂NHCO(CH₂)₁₈CH₄ | Erucyl stearamide |
| 22 | 17 | Dococenyl | Heptadecenyl | Dococenyloctadeceneneamide | CH₃(CH₂)₇HC=CH(CH₂)₁₂NHCO(CH₂)₇HC=CH(CH₂)₇CH₃ | Erucyl oleamide |
| 22 | 21 | Dococenyl | Heneicocenyl | Dococenyldococeneneamide | CH₃(CH₂)₇HC=CH(CH₂)₁₂NHCO(CH2)₁₁HC=CH(CH2)₇CH₃ | Erucyl erucamide |
| 24 | 11 | Tetracosyl | Undecyl | Tetracocyldodecaneamide | CH₃(CH₂)₂₃NHCO(CH₂)₁₀CH₃ | Lignoceryl lauramide |
| 24 | 17 | Tetracosyl | Heptadecyl | Tetracocyloctadecaneamide | CH₃(CH₂)₂₃NHCO(CH₂)₁₆CH₃ | Lignoceryl stearamide |

The amount of secondary amides may constitute 0.05-2.0 % by weight of the powder metal composition, preferably 0.05-1.0% by weight.

One embodiment of the invention concerns a powder metal composition comprising a lubricant and/or binder further comprising at least one primary amide in addition to the at least one secondary amide. The at least one primary amide is preferably a saturated or unsaturated fatty acid amide having 12-24, preferably 14-22 C-atoms and most preferably 16-22 C-atoms.

Especially preferred primary amides are stearic acid amide (stearamide), behenic acid amide (behenamide), eurcic acid amide (erucamide), palmitic acid amide (palmitamide) and arachidic acid amide (arachidamide).

The primary and secondary amides according to the invention are either commercially obtainable or may be produced from commercially obtainable material by the use of processes well known in the art.

The amount of primary and secondary amides may constitute a total of 0.05-2.0 % by weight of the powder metal composition, preferably 0.05-1.0% by weight.

The amount of the at least one primary amide may be 0.05-1.0% by weight and the amount of the at least one secondary amide may be 0.05-1.0% by weight for the embodiment of the invention comprising both types of amides.

The lubricant and/or binder may be added to the powder metal composition in the form of solid particles of each amide. The average particle size may vary, but is preferably less than 150 µm.

Alternatively, the lubricant and/or binder may be added to the powder metal composition as a molten and subsequently solidified particulate mixture of the amides. This may be accomplished by mixing the amides in a predetermined ratio, the mixture is then melted, cooled and subsequently milled to a lubricant powder.

The at least one secondary amide according to the invention may be used as a binder for obtaining a bonded mixture, wherein optional alloying elements and the at least one secondary amide are bonded to the iron-based powder. This may be achieved by mixing an iron-based powder with at least one secondary amide according to the invention, and heating the mixture to a temperature above the melting point of the at least one secondary amide. At least one primary amide may further be mixed into the above mentioned mixture and the heating temperature may then be lower than the melting point of the primary amide.

Apart from the lubricant and/or binder disclosed above, the powder metal composition according to the invention may, if so desired, contain other lubricants, such as zinc stearate, lithium stearate, EBS etc.

To accomplish a bonding of the powder metal composition according to the invention other types of bonding systems may be used such as alkydes, cellulose ester resins, hydroxyalkyl cellulose resins having 1-4 carbon atoms in the alkyl group, or thermoplastic phenolic resins.

As used in the description and the appended claims, the expression "iron-based" powder encompasses powder made up of pure iron, iron powder that has been pre-alloyed with other elements improving the strength, the hardening properties, the electromagnetic properties or other desirable properties of the end products and particles of iron mixed with particles of such alloying elements (diffusion annealed mixture or purely mechanical mixture). The alloying elements are copper, molybdenum, chromium, manganese, phosphorous, carbon in the form of graphite, nickel, silicon, boron, vanadium, titanium, aluminium, cobalt and tungsten, which are used either separately or in combination, e.g. in the form of compounds (Fe₃P and FeMo).

The iron based powders may be used for the preparation of soft magnetic parts and may, for this application, be electrically insulated. Electrical insulation of the powder particles may be made of an inorganic material. Especially suitable are the type of insulation disclosed in the US 6348265, which concerns particles of a base powder consisting of essentially pure iron having an insulating oxygen- and phosphorus-containing barrier. Insulated powder particles are available as Somaloy^{™} 500 and 550 from Hoganas AB, Sweden.

Apart from the iron-based powder and the lubricant and/or binder, the powder metal composition according to the invention may contain one or more additives selected from the group consisting of processing aids and hard phases.

The processing aids used in the powder metal composition may consist of talc, forsterite, manganese sulphide, sulphur, molybdenum disulphide, boron nitride, tellurium, selenium, barium difluoride and calcium difluoride, which are used either separately or in combination.

The hard phases used in the powder metal composition may consist of carbides of tungsten, vanadium, molybdenum, chromium, Al₂O₃, B₄C and various ceramic materials.

The invention further concerns a method of producing a green body comprising: compacting the powder metal composition according to the invention to a compacted body, wherein the composition comprises an iron based powder and a lubricant and/or binder comprising at least one secondary amide having the general formula: R₁-NH-CO-R2, wherein R₁ and R₂ are the same or different, straight or branched, saturated or unsaturated aliphatic hydrocarbon groups. The compacted body may be sintered or heat-treated.

With the aid of conventional techniques, the iron-based powder, the lubricant and/or binder and optional additives may be mixed to a substantially homogeneous powder composition before the compaction step.

The powder metal composition and/or the die may be preheated before the compaction.

The invention further concerns the use of at least one secondary amide, defined as above, as a lubricating and/or binding agent for iron or iron based powders.

A further embodiment of the invention concerns the use of at least one secondary amide, defined as above, as a die wall lubricant.

### Detailed description of the figure

Figure 1 shows stain formation of components after sintering due to the use of different lubricants.
1a) Ethylene bisstearamide (EBS);
1b) Oleyl palmitamide (a secondary amide according to the invention).

The invention will now be further described with the following unlimiting examples.

### Examples

In the following examples lubricants having the formulas disclosed in Table 2 below have been used.

**Table 2.**

| Chemical name | Structural formula* | Amide type |
|---|---|---|
| Ref: Ethylene* bis stearamide (EBS) | CH₃(CH₂)₁₆CONH(CH₂)₂NHCO(CH₂)₁₆CH₃ | bis amide |
| Stearamide (S) | CH₃(CH₂)₁₆CONH₂ | Primary |
| Arachidamide (A) | CH₃(CH₂₎₁₈CONH₂ | Primary |
| Erucamide (E) | CH₃(CH₂)₇CH=CH(CH₂)₁₁CONH₂ | Primary |
| Behenamide (B) | CH₃(CH₂)₂₀CONH₂ | Primary |
| Stearyl Stearamide (SS) | R1=C18:0 R2=C17:0 | Secondary |
| Erucyl Stearamide (ES) | R1=C22:1 R2=C17:0 | Secondary |
| Oleyl Palmitamide (OP) | R1=C18:1 R2=C15:0 | Secondary |
| Stearyl Erucamide (SE) | R₁=C18:0 R₂=C21:1 | secondary |
| Oleyl Stearamide (OS) | R₁=C18:1 R₂=C17:0 | secondary |
| Stearyl Oleamide (SO) | R=C18:0 R₂=C17:1 | secondary |

| | | |
|---|---|---|
| * The structural formulas for the secondary amides are referring to R₁-NH-CO-R₂ as previously described. * not part of the invention | | |

### Example 1

This example demonstrates the lubrication properties of different secondary amides and different combinations of secondary and primary amides, which are added as a powder in iron-based powder mixes.

Base powder ASC 100.29 (available from Hoganas AB, Sweden) was mixed with 0.5% by weight of graphite (uf-4 from Kropfmuhl) and 0.8% by weight of lubricants, according to Table 3 and 4, in a Lödige mixer for 2 minutes. Ethylene bisstearamide (EBS, available as Licowax TM from Clariant, Germany) was used as a reference. The lubricants had a particle size less than 150 µm. Compositions comprising both a secondary and a primary amide contained 50% of each amide (0.8% by weight of the total composition).

In order to measure the lubricating properties rings with an inner diameter of 45 mm, an outer diameter of 55 mm and a height of 10 mm were compacted at ambient temperature at three different compaction pressures (400, 600 and 800 MPa). During ejection of the compacted parts the ejection force was recorded. The green density of the parts was measured after ejection and the total ejection energy/enveloping area needed in order to eject the samples from the die was calculated.

The resulting ejection energies and densities are shown in Table 3 and 4. Lower ejection energies where achieved when using the powder metal composition according to the invention compared with the use of the reference composition comprising EBS.

**Table 3. Densities and ejection energies (secondary amides and reference).**

| Lubricant | Premixed | | | | | |
|---|---|---|---|---|---|---|
| | Green Density (g/cm³) | | | Ejection Energy (J/cm²) | | |
| | 400 MPa | 600 MPa | 800 MPa | 400 MPa | 600 MPa | 800 MPa |
| EBS (Ref) | 6.70 | 7.04 | 7.17 | 19.2 | 26.1 | 28.2 |
| SS | 6.72 | 7.06 | 7.19 | 17.6 | 24.7 | 27.9 |
| ES | 6.78 | 7.12 | 7.23 | 16.3 | 20.3 | 20.8 |
| OP | 6.78 | 7.14 | 7.25 | 16.7 | 21.3 | 20.3 |
| SE | 6.78 | 7.13 | 7.24 | 16.8 | 21.9 | 21.8 |
| OS | 6.78 | 7.13 | 7.24 | 17.7 | 21.3 | 20.5 |
| SO | 6.79 | 7.13 | 7.23 | 15.9 | 21.4 | 20.4 |

**Table 4. Densities and ejection energies (secondary + primary amides 1:1 and reference)**

| Lubricant | Premixed | | | | | |
|---|---|---|---|---|---|---|
| | Green Density (g/cm³) | | | Ejection Energy (J/cm²) | | |
| | 400 MPa | 600 MPa | 800 MPa | 400 MPa | 600 MPa | 800 MPa |
| EBS (Ref) | 6.70 | 7.04 | 7.17 | 19.2 | 26.1 | 28.2 |
| SS+E | 6.69 | 7.06 | 7.21 | 19.1 | 24.2 | 23.6 |
| OP+S | 6.70 | 7.06 | 7.19 | 18.2 | 22.1 | 22.3 |
| ES+S | 6.71 | 7.06 | 7.19 | 17.9 | 21.5 | 21.8 |
| ES+E | 6.72 | 7.11 | 7.23 | 17.8 | 20.7 | 19.0 |

### Example 2

The base powder ASC 100.29 was mixed with 2% by weight of Copper (-100µm), 0.8% by weight graphite and 0.8% by weight of lubricants (a) EBS or b) oleyl palmitamide) in a Lödige mixer for 2 minutes. The lubricants had a particle size less than 150 µm. In order to measure the stain formation after sintering of components, cylindrical components with a diameter of 64 mm and a height of 32 mm were compacted to a green density of 7.1 g/cm³ at ambient temperature. The weight of one cylinder was 700 g. The components were sintered in an atmosphere containing 90/10 N₂/H₂ at 1120°C for 15 minutes.

Photos of the components are shown in Figure 1a) Ethylene bisstearamide (EBS) and 1b) oleyl palmitamide, in which figure 1a) show stain formation in contrast to the part produced from the powder composition according to the present invention (1b) which has no stains.

### Example 3

This example demonstrates the lubrication properties of different combinations of secondary and primary amides, which have been melted together, cooled and milled before being mixed with iron-based powder mixes.

The lubricant combinations were made according to following method: The mixed lubricants, 50% primary and 50% secondary amide, were melted together at 80-110°C and then cooled. Then the materials were milled to a mean particle size of below 150µm.

The base powder ASC100.29 was mixed with 0.5 % by weight of graphite and 0.8 % by weight of lubricant combination (see Table 5), in a Lödige mixer for 2 minutes. In order to measure the lubricating properties rings with inner diameter of 45 mm, outer diameter 55 mm and a height 10 mm were compacted at three different compaction pressures, 400, 600 and 800 MPa at ambient temperature. The resulting ejection energies and densities are shown in Table 5.

**Table 5. Densities and ejection energies (secondary + primary amides and reference).**

| Lubricant | Melted and solidified | | | | | |
|---|---|---|---|---|---|---|
| | Green Density (g/cm³) | | | Ejection Energy (J/cm²) | | |
| | 400 MPa | 600 MPa | 800 MPa | 400 MPa | 600 MPa | 800 MPa |
| EBS (Ref) | 6.70 | 7.04 | 7.17 | 19.2 | 26.1 | 28.2 |
| SS+E | 6.70 | 7.06 | 7.20 | 18.8 | 22.4 | 22.6 |
| OP+S | 6.71 | 7.07 | 7.20 | 18.5 | 23.2 | 24.4 |
| ES+S | 6.71 | 7.07 | 7.20 | 18.9 | 22.7 | 23.5 |
| ES+E | 6.70 | 7.07 | 7.20 | 17.2 | 19.8 | 18.0 |

When comparing the test results in Table 5 it can be seen that samples produced from the powder metal composition according to the invention show lower ejection energies compared to samples produced from the known lubricant EBS.

### Example 4

This example demonstrates the lubricating and binding properties of different combinations of amides in powder metal compositions.

The lubricants had a particle size less than 150 µm. The base powder ASC100.29 was mixed with 2% by weight Cu-100, 0.8 % by weight of graphite and 0,8 % by weight of lubricant/binder combination according to Table 6, in a Lödige mixer for 2 minutes. The mixture with EBS was kept as reference while the mixtures comprising amides were heated to a temperature above the melting point of the secondary amide but below the melting point of the primary amide during mixing in another mixer followed by cooling to accomplish bonding of the additives to the iron powder. In this mixture the secondary amide will thus act as a binder and the primary amide will act as a lubricant. The melting temperatures of the amides are disclosed in Table 7.

Further, the ejection energy was measured on rings having an outer diameter of 55 mm and an inner diameter of 45 mm and a height of 10 mm compacted at three different compaction pressures, 400, 600 and 800 MPa at ambient temperature. The resulting ejection energies and green densities are shown in Table 8.

**Table 6. Lubricant/binder combinations for example 4.**

| Secondary amide | Primary amide |
|---|---|
| 0.2% by weight | 0.6% by wt |
| ES | B |
| OP | S |
| OP | B |
| EBS (Ref 1) (0.8% by wt) | |

**Table 7. Melting temperatures of the amides.**

| Amide | Melting temperature(°C) |
|---|---|
| ES | 72.9 |
| OP | 66.9 |
| B | 101.9 |
| S | 106.6 |

**Table 8. Densities and ejection energies (primary + secondary amides and reference).**

| Binder/Lubricant | Melt bonded | | | | | |
|---|---|---|---|---|---|---|
| | Green Density (g/cm³) | | | Ejection Energy (J/cm²) | | |
| | 400 MPa | 600 MPa | 800 MPa | 400 MPa | 600 MPa | 800 MPa |
| ES+B | 6.75 | 7.06 | 7.19 | 18.5 | 24.6 | 28.1 |
| OP+S | 6.73 | 7.09 | 7.18 | 19.3 | 26.6 | 28.3 |
| OP+B | 6.77 | 7.08 | 7.19 | 19.9 | 25.3 | 27.1 |
| EBS (Ref) | 6.74 | 7.06 | 7.17 | 21.4 | 30.8 | 32.8 |

Samples produced with the aid of the lubricant/binder according to the invention show lower ejection energies compared to samples produced with the lubricant used as reference, i.e. EBS. Use of the powder composition comprising the lubricant/binder according to the invention resulted in compacted sintered parts (sintered in 90/10 N₂/H₂ at 1120°C for 30 minutes) with excellent surface finishes, i.e. essentially without scratches and no stain formation.

### Example 5

A coarse soft magnetic iron-based powder, wherein the particles are surrounded by an inorganic insulation was mixed with secondary amide lubricant according to Table 9. As reference lubricants the known substances Zinc-stearate and EBS were used. The particle size distribution of the used iron-based powder is disclosed in Table 10.

The obtained mixes were transferred to a die and compacted into cylindrical test samples (50 g) having a diameter of 25 mm, in an uniaxial press movement at a compaction pressure of 1100 MPa. The die material used was conventional tool steel. During ejection of the compacted samples the ejection force was recorded. The total ejection energy/enveloping area needed in order to eject the samples from the die was calculated.

The results of the measurements regarding ejection energy, green density and surface appearance in the green state are shown in Table 9. Use of the powder metal compositions according to the invention resulted in that compacted components with excellent surface appearance and lower ejection energies were achieved compared with the reference compositions.

**Table 9. Densities, ejection energies and surface appearance.**

| Mix no | Lubricant (0.2 wt%) | Ejection energy (J/cm²) | Green Density (g/cm³) | Surface appearance |
|---|---|---|---|---|
| 1 | ES | 76 | 7.65 | Perfect |
| 2 | SE | 71 | 7.66 | Perfect |
| 3 | SS | 78 | 7.63 | Perfect |
| 4 | OP | 76 | 7.66 | Perfect |
| Ref 1 | Zinc stearate | 117 | 7.66 | Not acceptable |
| Ref 2 | EBS | 113 | 7.64 | Perfect |

**Table 10**

| Particle size (µm) | Coarse powder (wt%) |
|---|---|
| >425 | 0.1 |
| 425-212 | 64.2 |
| 212-150 | 34.1 |
| 150-106 | 1.1 |
| 106-75 | 0.3 |
| 45-75 | 0.2 |
| <45 | 0 |

## Claims

1. Powder metal composition comprising an iron based powder selected from pure iron, iron powder pre-alloyed, diffusion annealed or mechanically mixed with one or more alloying elements selected from Cu, Mo, Cr, Mn, P, C in the form of graphite, Ni, Si, B, V, Ti, Al, Co, W, or mixtures thereof and a lubricant and/or binder comprising 0.05-2% by weight of at least one secondary amide of the general formula:
R₁-NH-CO-R₂
**characterised in that** R₁ and R₂ are the same or different, straight or branched, saturated or unsaturated aliphatic hydrocarbon groups.

2. Composition according to claim 1, wherein R₁ and R₂ independently include 10 to 24 carbon atoms.

3. Composition according to claims 1 or 2, wherein R₁ and R₂ are selected from the group consisting of alkyl and alkenyl.

4. Composition according to claim 3, wherein the alkyl groups are chosen from decyl, undecyl, dodecyl, tridecyl, tetradecyl, pentadecyl, hexadecyl, heptadecyl, octadecyl, nonadecyl, eicosyl, heneicosyl, docosyl, tricosyl, tetracosyl.

5. Composition according to claim 3, wherein the alkenyl groups are chosen from decenyl, undecenyl, dodecenyl, tridecenyl, tetradecenyl, pentadecenyl, hexadecenyl, heptadecenyl, octadecenyl, nonadecenyl, eicosenyl, heneicosenyl, docosenyl, tricosenyl, tetracosenyl.

6. Composition according to claim 1, wherein the secondary amide is chosen from oleyl palmitamide, stearyl stearamide, oleyl stearamide, stearyl oleamide, oleyl oleamide, stearyl erucamide, oleyl erucamide, erucyl stearamide, erucyl oleamide, erucyl erucamide, lignoceryl lauramide, lignoceryl stearamide.

7. Composition according to claim 1, further comprising at least one primary amide.

8. Composition according to claim 7, wherein the primary amide is an amide of a saturated or unsaturated, straight fatty acid having 12-24 carbon atoms.

9. Composition according to claim 7, wherein the primary amide is selected from the group consisting of palmitamide, stearamide, arachidamide, behenamide and erucamide.

10. Composition according to any one of claims 1-9, wherein the lubricant is particulate.

11. Composition according to any one of claims 7-9, wherein the lubricant comprises a molten and subsequently solidified particulate mixture of the at least one secondary amide and the at least one primary amide.

12. Composition according to any one of claims 1-9, wherein the composition is a bonded mixture.

13. Composition according to claim 12, wherein at least one secondary amide is used as a binding agent.

14. Composition according to any one of claims 1-9, wherein the iron-based particles are surrounded by an insulating inorganic coating.

15. Method of producing a green body comprising:
compacting the powder metal composition according to any one of claims 1-9 to a compacted body.

16. Method according to claim 15, further comprising a heat treatment or sintering step.

17. Method of producing a bonded iron-based powder composition comprising:
- mixing an iron-based powder with at least one secondary amide according to any one of claims 1-9;
- heating the mixture to a temperature above the melting point of the at least one secondary amide.

18. Method according to claim 17, wherein the mixture further comprises at least one primary amide and wherein the heating temperature is lower than the melting point of the primary amide.

19. Use of a lubricant and/or binder according to any one of claims 1-9 as a lubricating and/or binding agent for iron based powders.

20. Use of a lubricant according to any one of claims 1-9 as a die wall lubricant.

## Patentansprüche

1. Pulvermetallzusammensetzung, die ein Pulver auf Eisenbasis ausgewählt unter reinem Eisen, Eisenpulver, das mit einem oder mehreren legierenden Elementen vorlegiert, diffusionsgeglüht oder mechanisch gemischt wird, die unter Cu, Mo, Cr, Mn, P, C in Form von Graphit, Ni, Si, B, V, Ti, Al, Co, W oder Mischungen derselben ausgewählt werden, und ein Gleitmittel und/oder Bindemittel umfasst, das 0,05 - 2 Gew.-% mindestens eines sekundären Amids der allgemeinen Formel:
R₁-NH-CO-R₂
umfasst, **dadurch gekennzeichnet, dass** R₁ und R₂ gleiche oder verschiedene, geradkettige oder verzweigte, gesättigte oder ungesättigte aliphatische Kohlenwasserstoffgruppen sind.

2. Zusammensetzung nach Anspruch 1, wobei R₁ und R₂ unabhängig 10 bis 24 Kohlenstoffatome umfassen.

3. Zusammensetzung nach Anspruch 1 oder Anspruch 2, wobei R₁ und R₂ aus der Gruppe ausgewählt werden bestehend aus Alkyl und Alkenyl.

4. Zusammensetzung nach Anspruch 3, wobei die Alkylgruppen unter Decyl, Undecyl, Dodecyl, Tridecyl, Tetradecyl, Pentadecyl, Hexadecyl, Heptadecyl, Octadecyl, Nonadecyl, Eicosyl, Heneicosyl, Docosyl, Tricosyl, Tetracosyl ausgewählt werden.

5. Zusammensetzung nach Anspruch 3, wobei die Alkenylgruppen unter Decenyl, Undecenyl, Dodecenyl, Tridecenyl, Tetradecenyl, Pentadecenyl, Hexadecenyl, Heptadecenyl, Octadecenyl, Nonadecenyl, Eicosenyl, Heneicosenyl, Docosenyl, Tricosenyl, Tetracosenyl ausgewählt werden.

6. Zusammensetzung nach Anspruch 1, wobei das sekundäre Amid unter Oleylpalmitat, Stearylstearamid, Oleylstearamid, Stearyloleamid, Oleyloleamid, Stearylerucamid, Oleylerucamid, Erucylstearamid, Erucyloleamid, Erucylerucamid, Lignoceryllauramid, Lignocerylstearamid ausgewählt wird.

7. Zusammensetzung nach Anspruch 1, des Weiteren mindestens ein primäres Amid umfassend.

8. Zusammensetzung nach Anspruch 7, wobei das primäre Amid ein Amid einer gesättigten oder ungesättigten, geradkettigen Fettsäure ist, die 12 - 24 Kohlenstoffatome aufweist.

9. Zusammensetzung nach Anspruch 7, wobei das primäre Amid aus der Gruppe ausgewählt wird bestehend aus Palmitamid, Stearamid, Arachidamid, Behenamid und Erucamid.

10. Zusammensetzung nach einem der Ansprüche 1 - 9, wobei das Gleitmittel teilchenförmig ist.

11. Zusammensetzung nach einem der Ansprüche 7 - 9, wobei das Gleitmittel eine geschmolzene und daraufhin verfestigte teilchenförmige Mischung des mindestens einen sekundären Amids und des mindestens einen primären Amids umfasst.

12. Zusammensetzung nach einem der Ansprüche 1 - 9, wobei die Zusammensetzung eine gebundene Mischung ist.

13. Zusammensetzung nach Anspruch 12, wobei mindestens ein sekundäres Amid als Bindemittel verwendet wird.

14. Zusammensetzung nach einem der Ansprüche 1 - 9, wobei die Teilchen auf Eisenbasis von einer isolierenden anorganischen Beschichtung umgeben sind.

15. Verfahren zum Herstellen eines grünen Körpers, umfassend:
das Verdichten der Pulvermetallzusammensetzung nach einem der Ansprüche 1 - 9 zu einem verdichteten Körper.

16. Verfahren nach Anspruch 15, des Weiteren einen Hitzebehandlungs- oder Sinterschritt umfassend.

17. Verfahren zum Herstellen einer gebundenen Pulverzusammensetzung auf Eisenbasis, umfassend:
- das Mischen eines Pulvers auf Eisenbasis mit mindestens einem sekundären Amid nach einem der Ansprüche 1 - 9;
- das Erhitzen der Mischung auf eine Temperatur über dem Schmelzpunkt des mindestens einen sekundären Amids.

18. Verfahren nach Anspruch 17, wobei die Mischung des Weiteren mindestens ein primäres Amid umfasst und wobei die Erhitzungstemperatur niedriger als der Schmelzpunkt des primären Amids ist.

19. Verwendung eines Gleitmittels und/oder Bindemittels nach einem der Ansprüche 1 - 9 als Gleitmittel und/oder Bindemittel für Pulver auf Eisenbasis.

20. Verwendung eines Gleitmittels nach einem der Ansprüche 1 - 9 als Matrizenwandgleitmittel.

## Revendications

1. Composition métallique en poudre comprenant une poudre à base de fer choisie parmi le fer pur, la poudre de fer préalliée, recuite par diffusion ou mécaniquement mélangée avec un ou plusieurs éléments d'alliage choisis parmi Cu, Mo, Cr, Mn, P, C sous la forme de graphite, Ni, Si, B, V, Ti, AI, Co, W ou des mélanges de ceux-ci et un lubrifiant et/ou liant comprenant 0,05 à 2 % en masse d'au moins un amide secondaire de formule générale :
R₁-NH-CO-R₂
**caractérisée en ce que** R₁ et R₂ sont des groupes hydrocarbures aliphatiques identiques ou différents, linéaires ou ramifiés, saturés ou insaturés.

2. Composition selon la revendication 1, dans laquelle R₁ et R₂ comprennent, indépendamment l'un de l'autre, 10 à 24 atomes de carbone.

3. Composition selon la revendication 1 ou 2, dans laquelle R₁ et R₂ sont choisis dans le groupe constitué par l'alkyle et l'alcényle.

4. Composition selon la revendication 3, dans laquelle les groupes alkyles sont choisis parmi le décyle, l'undécyle, le dodécyle, le tridécyle, le tétradécyle, le pentadécyle, l'hexadécyle, l'heptadécyle, l'octadécyle, le nonadécyle, l'éicosyle, l'henéicosyle, le docosyle, le tricosyle et le tétracosyle.

5. Composition selon la revendication 3, dans laquelle les groupes alcényles sont choisis parmi le décényle, l'undécényle, le dodécényle, le tridécényle, le tétradécényle, le pentadécényle, l'hexadécényle, l'heptadécényle, l'octadécényle, le nonadécényle, l'éicosényle, l'henéicosényle, le docosényle, le tricosényle et le tétracosényle.

6. Composition selon la revendication 1, dans laquelle l'amide secondaire est choisi parmi le palmitamide d'oléyle, le stéaramide de stéaryle, le stéaramide d'oléyle, l'oléamide de stéaryle, l'oléamide d'oléyle, l'érucamide de stéaryle, l'érucamide d'oléyle, le stéaramide d'érucyle, l'oléamide d'érucyle, l'érucamide d'érucyle, le lauramide de lignocéryle et le stéaramide de lignocéryle.

7. Composition selon la revendication 1, comprenant en outre au moins un amide primaire.

8. Composition selon la revendication 7, dans laquelle l'amide primaire est un amide d'un acide gras linéaire saturé ou insaturé ayant 12 à 24 atomes de carbone.

9. Composition selon la revendication 7, dans laquelle l'amide primaire est choisi dans le groupe constitué par le palmitamide, le stéaramide, l'arachidamide, le béhénamide et l'érucamide.

10. Composition selon l'une quelconque des revendications 1 à 9, dans laquelle le lubrifiant est particulaire.

11. Composition selon l'une quelconque des revendications 7 à 9, dans laquelle le lubrifiant comprend un mélange particulaire fondu puis solidifié d'au moins un amide secondaire et d'au moins un amide primaire.

12. Composition selon l'une quelconque des revendications 1 à 9, dans laquelle la composition est un mélange lié.

13. Composition selon la revendication 12, dans laquelle au moins un amide secondaire est utilisé comme agent liant.

14. Composition selon l'une quelconque des revendications 1 à 9, dans laquelle les particules à base de fer sont entourées d'un revêtement inorganique isolant.

15. Procédé de production d'une ébauche crue comprenant :
le compactage de la composition métallique en poudre selon l'une quelconque des revendications 1 à 9 en une ébauche comprimée.

16. Procédé selon la revendication 15, comprenant en outre une étape de traitement thermique ou de frittage.

17. Procédé de production d'une composition de poudre à base de fer liée comprenant :
- le mélange d'une poudre à base de fer avec au moins un amide secondaire selon l'une quelconque des revendications 1 à 9 ;
- le chauffage du mélange à une température supérieure au point de fusion d'au moins un amide secondaire.

18. Procédé selon la revendication 17, dans lequel le mélange comprend en outre au moins un amide primaire et dans lequel la température de chauffage est inférieure au point de fusion de l'amide primaire.

19. Utilisation d'un lubrifiant et/ou liant selon l'une quelconque des revendications 1 à 9 comme agent lubrifiant et/ou liant pour les poudres à base de fer.

20. Utilisation d'un lubrifiant selon l'une quelconque des revendications 1 à 9 comme lubrifiant pour parois de filières.
